

## 1

3,071,547

## MIXED-SALT LUBRICANTS

Arnold J. Morway, Clark, N.J., assignor to Esso Research and Engineering Company, a corporation of Delaware  
No Drawing. Filed Aug. 23, 1960, Ser. No. 51,255  
5 Claims. (Cl. 252—39)

This invention relates to fluid and semi-fluid lubricating oil compositions having good extreme pressure and antiwear properties. Particularly, the invention relates to a lubricant comprising lubricating oil containing an anhydrous mixture of metal salts of low molecular weight carboxylic acid and moderate molecular weight carboxylic acid, which compositions are useful for the lubrication of the upper cylinders of marine diesel engines.

This application is a continuation-in-part of U.S. patent application Serial Number 498,740, by Arnold J. Morway, filed April 1, 1955, and now abandoned.

Marine diesel engines have become widespread in their use. In these engines there has always been a serious wear problem with regard to the piston, the piston rings and the surface of the cylinder liner. This problem of wear has been aggravated by the recent growing tendency to use low cost residual type fuel oils. These residual fuel oils contain 2 to 4 wt. percent sulfur, as compared to distillate oils which generally head under 1.5% sulfur. However, these residual fuels represent a large economic saving over the previously used distillate fuel oils. Unfortunately, because of their high sulfur content, the residual fuels result in increasing the liner and cylinder wear from 50 to 500% over the wear previously encountered with distillate fuels. This increased wear is primarily due to acids formed by the combustion of the sulfur, which acids corrode the steel surfaces of the engine.

In lubricating these diesel engines, a fluid or semi-fluid lubricant is sprayed directly onto the cylinder upon each stroke of the piston by means of a centralized force-feed lubrication system. The lubricant is to a large extent consumed during each stroke of the piston, thereby requiring continuous application of the lubricant.

In order to be suitable for such lubrication use, it has been determined that the lubricant should have a fluid or semifluid consistency. This is desired in order that the lubricant may be readily pumped through the aforementioned forced lubrication systems normally associated with marine diesel engines and will spread or wet the piston sufficiently during each stroke to achieve an overall coating on the piston surface. It has been further found that extreme pressure characteristics are necessary, since the pressure of the piston rings against the cylinder liner is very considerable. Thus, such lubricants should be able to carry at least 6 weights in the standard Almen extreme pressure test under gradual loading. A third requirement of such lubricants is that they have good antiwear properties. Because of the giant size of the pistons and cylinders used in such engines (e.g. piston and cylinder diameters of 36 to 60 inches are common), wear is a serious problem. Once the cylinder liner has worn more than about 0.6% of its diameter, it is necessary that it be replaced. In a typical marine engine of 8 to 16 cylinders such replacement cost may run in the order of several thousand dollars per cylinder. Wear of the piston and rings are also an expensive problem. It is, therefore, essential that their wear be minimized and for this purpose lubricants to be acceptable should have wear scar diameters of 0.19 to 0.28 mm. as measured

## 2

in the Shell 4 ball wear test under relatively severe conditions of load versus times, i.e. under a 10 kilogram load, at 1800 r.p.m. for 1 hour at 77° F. The fourth major requirement of a lubricant of this type is that it should be able to minimize the wear due to corrosiveness caused by the degradation products of the oil and particularly of the sulfur. A fifth important requirement is that the lubricant be storage stable, even when subject to long periods of vibration as occurs during storage in a ship's engine room and in the presence of minor amounts of moisture.

It has been found that requirements for the above type of lubricant can be obtained by thickening oil with 5 to 12, preferably 6 to 8 wt. percent of total thickener comprising calcium salt of acetic acid or its anhydride in combination with calcium salt of  $C_7$  to  $C_{19}$  fatty acids in a molar equivalent ratio of about 11.5:1 to 25:1 of said acetic acid or anhydride per mole of said higher fatty acid. At molar ratios of less than 11.5:1 it has been found that insufficient extreme pressure and antiwear properties are obtained and that the lubricant requires a larger amount of salt per amount of oil as well as having a viscosity that is excessive for pumping and spraying onto the piston. At molar ratios greater than 25:1, it has been found that the lubricant is unsuitable because of storage instability since the salts will settle out of the oil leading to clogging of the lubrication system and the lubricant tends to become more susceptible to water solubility, i.e. poor sight glass performance.

30 The intermediate molecular weight acids used in preparing the thickener are those aliphatic straight chain monocarboxylic acids containing from about 7 to 10 carbon atoms. Either saturated or unsaturated fatty acids may be utilized, though the saturated fatty acids are preferred. The corresponding branched chain acids are not suitable since they result in unstable lubricants in which the salts readily separate from the oil. Intermediate molecular weight straight chain monocarboxylic acids coming within the above prescriptions are exemplified by heptanoic (enanthic), octanoic (caprylic), nonanoic (pelargonic) and decanoic (capric). Commercial mixtures of these intermediate molecular weight carboxylic acids having an average saponification of from about 310 to 440, preferably 320 to 420 can also be employed.

40 The metal component of the mixed salt composition is preferably calcium since it results in the production of stable lubricants having excellent load carrying and antiwear characteristics even without the use of conventional extreme pressure and stabilizing agents. The other alkaline earth metals such as barium, strontium and magnesium are inferior to calcium in these respects as are the alkali metals, e.g. sodium, potassium and lithium.

45 The anhydrous mixture of calcium salts of the invention may be prepared by coneutralization of a mixture of the acids with suitable bases, particularly the hydroxides and/or carbonates of calcium. The coneutralization step may be carried out in situ in the oil menstruum to which the mixture of salts is to be applied in actual use.

50 The maximum temperature at which coneutralization is carried out or the temperature to which the coneutralized material is heated will generally be in the range of about 250° to about 350° F. The salt mixture should be heated until anhydrous, i.e. there is no free or unbound water present. If the acids are coneutralized then it is generally desirable to use a slight excess of base, e.g. lime, in order

to form a slightly alkaline final product, e.g. 0.05 to 0.2 wt. percent alkalinity as measured in terms of NaOH. This alkalinity acts to neutralize corrosive acids formed by degradation of the lubricant during use and also imparts conditions of greater stability.

If the acids are to be conneutralized with commercial lime, it has been found that sedimentation can be reduced by first partially neutralizing the acids with lime, cooking for about 2 to 4 hours, below 225° F., then adding the remainder of the lime to complete the neutralization and in fact, form a slightly alkaline product. By this method, the CaCO<sub>3</sub> which is present in commercial lime in quantities up to 5 wt. percent will be forced to substantially complete reaction with the acids. Otherwise, the calcium hydroxide will react preferentially to the calcium carbonate so that the desired excess alkalinity will be primarily due to the calcium carbonate. Unfortunately, the unreacted calcium carbonate tends to settle out and results in sedimentation of the final product.

However, the conneutralization methods outlined above are not necessary as long as the two classes of salts are present when the composition is heated to dehydration temperatures within the range of 250° F. to 350° F. Thus, the mixture of calcium salts of the invention may also be prepared by separately preforming in aqueous media at least a portion or all of the low molecular weight acetate salt and/or the intermediate molecular weight carboxylic acid salt and heating them together under substantially dehydration conditions. The salts may also be intimately mixed prior to the heating step.

The use of preformed metal salts may also be desirable for other considerations. The production of the mixtures of calcium salts here involved requires large amounts of low molecular weight carboxylic acids, particularly, acetic acid or its anhydride. These acids may be purchased in carload or tank car lots; but they require tankage with piping to the kettles and special handling precautions to prevent them from solidifying in the piping and from corroding the tanks and pipes. By supplying a portion or all of the required low molecular weight acid in the form of preformed metal salt, for example, calcium acetate, the drawbacks just mentioned may be minimized or eliminated. These advantages may be obtained by replacing about 30 to 80%, preferably, at least about 50%, of the free acid and its stoichiometric equivalent of free base with the preformed metal salt.

In general, the lubricating oil should have a viscosity within the range of about 100 to 2,500 SUS at 100° F. and about 35 to 200 SUS at 210° F., a pour point of about +20° to -75° F., and a flash point of about 350° to 650° F. A viscosity index of 100 or higher is also desirable, though mineral oils having a lower viscosity index can be desirably employed. The lubricating oil base can also consist of a blend of about 50-85 wt. percent of a relatively low viscosity oil of 30 to 70 SUS at 210° F., and about 15-50 wt. percent of a relatively high viscosity oil of 200 to 2,500 SUS at 100° F. Mineral oil mixtures of 20 to 50 wt. percent naphthenic oil of V.I. of 30 to 60 and viscosity of 50 to 80 SUS at 210° F. with 80 to 50 wt. percent of solvent extract oil of V.I. of 0 to -100 and viscosity of 100 to 175 SUS at 210° F. have been found very desirable in preventing fouling of sight glasses which are normally used in marine diesel forced-feed systems. The solvent extract oil used in this type of formulation can be prepared by solvent extraction of paraffinic or mixed base lubricating oil with phenol, furfural, nitrobenzene, etc. as is well known in the art.

Synthetic non-hydrocarbon oils, such as silicone oils do not give the same results as mineral oils because of their high wear imparting properties which are modified but not sufficiently overcome by the calcium mixed-salt thickener. Furthermore, synthetic oils such as polysilicones are unduly expensive since the lubricant is continuously consumed during use in marine diesel engines, rather than being recirculated.

Various additives can be added to the finished lubricant in amounts of 0.1 to 10.0 wt. percent, based on the weight of the finished lubricant. Among additives that can be added are corrosion inhibitors such as sodium nitrite, lanolin, wool grease stearine; antioxidants such as phenyl  $\alpha$ -naphthylamine; auxiliary extreme pressure agents; dyes; etc. The temperature at which the mixture of calcium salts is prepared or heated is an important feature of the present invention, since it determines in a large measure the physical as well as the chemical characteristics of the resulting products.

In accordance with this invention maximum dehydration temperatures of about 250° to 350° F., preferably, about 300° to 320° F., are employed to prepare the anhydrous (i.e. dry) mixtures of salts. At either lower or higher temperature the nature of the reaction products differs significantly from the products obtained at the preferred dehydration temperature with regard to such properties as appearance, stability, etc. Heating to high temperatures, e.g. about 400° to 550° F. will result in instability or undue thickening of the lubricant per given amount of salt, while heating at temperatures below 250° F. does not completely eliminate free water, which has a tendency to form solid (hydrous) products which are most undesirable.

The finished lubricant will comprise a major amount of lubricating oil and about 5 to 12, preferably 6 to 8 wt. percent of the mixed salt combination. For economy purposes in heating during large scale manufacture, concentrates of 35 to 50 wt. percent of the mixed salts in oil can be made by the in situ preparation technique and then the concentrate is diluted with additional oil to form the finished lubricant. This dilution is readily made by adding the additional oil and mixing in the kettle or by using a pump around system where the lubricant is passed from the kettle to a pump and then back to the kettle until completely mixed. Both the concentrate and finished lubricant can be homogenized in a Morehouse mill, Charlotte mill, Gaulin homogenizer, etc.

#### EXAMPLE I

(All parts by weight)

A grease was prepared by charging 88.72 parts of mineral lubricating oil having a viscosity of 70 SUS at 210° F. and 4.13 parts of hydrated lime to a steam heated kettle and slurried together to form a smooth uniform slurry. Steam was then passed into the kettle jacket, and the ingredients warmed to 135° F. Then 5.63 parts of glacial acetic acid and 1.34 parts of caprylic acid (commercial grade—Saponification No. 327 mg. KOH per gm.) was added and the temperature was raised to about 300° F. and maintained at this temperature for about 3 hours. The mixture was then cooled to 200° F. where 0.18 part of phenyl alpha-naphthylamine was added as an antioxidant. The mixture was further cooled to room temperature while stirring continuously. The resulting lubricant composition was then homogenized by passage through a Gaulin homogenizer operating at 5000 p.s.i. This product contained calcium salt of acetic acid to calcium salt of caprylic acid in a molar ratio of 12 to 1 and was employed as a marine diesel engine upper cylinder lubricant where it effectively reduced cylinder liner wear and minimized acid corrosion.

The above product was tested in a total of seven ships being used in the No. 4 cylinder of each marine diesel engine, while for comparison purposes the No. 1 cylinder of each of said engines was lubricated with a conventional straight mineral oil marketed as a marine diesel cylinder lubricant. All cylinder liners were new at the start of the test. The following table summarizes the result obtained, listing the engines tested, the type fuel that they operated upon, the length of the test and the average cylinder wear obtained in terms of inches/1000 hours' operation together with the wear reduction.

Table I  
COMPARATIVE SERVICE PERFORMANCE

| Test ship service                 | Tanker 1                                         | Tanker 2                                         | Passenger 3                                 | Passenger 4                               | Tanker 5                                          | Tanker 6                                      | Tanker 7                                      |
|-----------------------------------|--------------------------------------------------|--------------------------------------------------|---------------------------------------------|-------------------------------------------|---------------------------------------------------|-----------------------------------------------|-----------------------------------------------|
| Test ship number                  | 1                                                | 2                                                | 3                                           | 4                                         | 5                                                 | 6                                             | 7                                             |
| Engine                            | 2 Burn. & Wain, 8-cyl., 2-stroke, single-acting. | 2 Burn. & Wain, 9-cyl., 2-stroke, single-acting. | 2 Doxford, 6-cyl., 2-stroke, single-acting. | 2 Fiat, 10-cyl., 2-stroke, single-acting. | Harland & Wolff, 6-cyl., 4-stroke, single-acting. | Sun-Doxford, 5-cyl., 2-stroke, single-acting. | Sun-Doxford, 5-cyl., 2-stroke, single-acting. |
| Bore/stroke                       | 740/1,400 mm                                     | 740/1,400 mm                                     | 670/2,320 mm                                | 750/1,320 mm                              | 740/1,500 mm                                      | 813/2,410 mm                                  | 813/2,410 mm                                  |
| Brake horsepower                  | 7,000 at 118 r.p.m.                              | 7,100 at 112 r.p.m.                              | 6,300 at 105 r.p.m.                         | 7,750 at 120 r.p.m.                       | 3,300 at 110 r.p.m.                               | 7,500 at 94 r.p.m.                            | 7,500 at 94 r.p.m.                            |
| Fuel:                             |                                                  |                                                  |                                             |                                           |                                                   |                                               |                                               |
| Sulfur, weight percent.           | 3.3-4.2                                          | 2.2-3.3                                          | 3.0                                         | 2.2-3.5                                   | 3.1-4                                             | 1.2-2.3                                       | 1.2-2.3                                       |
| Viscosity, SSU at 100° F.         | 1,800-2,700                                      | 750-1,500                                        | 700                                         | 450-1,000                                 | 900-1,100                                         | 400-4,000                                     | 490-4,000                                     |
| Test Hours                        | 2,500-5,600                                      | 5,000                                            | 500-1,500                                   | 3,000                                     | 2,000                                             | 10,000                                        | 5,400                                         |
| Avg. cyl. wear inches/1,000 hrs.: |                                                  |                                                  |                                             |                                           |                                                   |                                               |                                               |
| Prior commercial lubricant.       | 0.019                                            | 0.021                                            | 0.025                                       | 0.016                                     | 0.008                                             | 0.020                                         | 0.020                                         |
| Lubricant of Ex. I.               | 0.013                                            | 0.004                                            | 0.006                                       | 0.002                                     | No measurable wear in 2,000 hr.                   | 0.008                                         | 0.010                                         |
| Wear reduction, percent.          | 30                                               | 84                                               | 74                                          | 90                                        |                                                   | 60                                            | 50                                            |

In the table, Tanker 1 had two Burmeister and Wain engines, each having a bore of 740 mm., a stroke of 1400 mm. and developing 7000 brake horsepower. Both engines were operated on high sulfur content residual fuel oil. One engine was tested for 2500 hours and the other for 5600 hours. The average liner wear of the No. 1 cylinder of the two engines using a commercial straight mineral oil marine diesel lubricant was 0.019 inch per 1000 hours' operation. The average liner wear of the No. 4 cylinder of the two engines, using the lubricant of Example I, was 0.013 inch per 1000 hours' operation. The composition of the invention thus gave 30% less wear than the commercial oil, which was one of the best available for marine diesel use. Even better results were obtained in the other ships under test.

Usually when cylinder liner wear exceeds a total of 0.6% of the bore of the cylinder, it is necessary to replace the cylinder liner. Thus, for an engine of 700 mm. bore, the cylinder liner would generally be removed after wear of 4.2 mm. or about 0.12 inch. For an average ship having two engines of 8 cylinders each or a total of 16 cylinders, this replacement cost will be about \$40,000 to \$60,000 plus the cost of the downtime of the ship. It is thus seen that the percent wear reduction shown in the preceding table represents a very substantial economic saving.

#### EXAMPLE II

A series of lubricants (A to E) was prepared to demonstrate the criticality of the mol ratio of the acetate to salt of the higher fatty acid. These lubricants were prepared as follows: About 99% of the hydrated lime was dispersed in about a sixth of the mineral oil. Then glacial acetic acid was slowly added to the lime-oil dispersion and next the capric acid was added. The mixture was continuously mixed while both acids were added and the temperature maintained below 200° F. The remaining 1% lime was added to complete the neutralization of the acids. External heating was next applied and the composition was heated to 320° F. until all the water of reaction had been evaporated and a dry composition formed. The composition was then cooled to about 200° F. where phenyl  $\alpha$ -naphthylamine was added as an oxidation inhibitor. The remainder of the oil was added and the composition homogenized in a Charlotte mill.

The capric acid used above was a commercial acid obtained from coconut oil and having a saponification number of about 320.

The compositions prepared and their physical properties are summarized in the following table.

Table II  
EFFECT OF MOL RATIO OF ACETIC ACID TO  
INTERMEDIATE MOL. WT. ACID

|    |                                                                    | A     | B     | C      | D     | E     |
|----|--------------------------------------------------------------------|-------|-------|--------|-------|-------|
| 30 | Formulation:                                                       |       |       |        |       |       |
|    | Glacial acetic acid, weight percent                                | 4.00  | 4.00  | 4.00   | 4.00  | 4.00  |
|    | Capric acid, weight percent                                        | 1.19  | 1.14  | 0.92   | 0.76  | 0.60  |
|    | Hydrated lime, weight percent                                      | 3.15  | 3.10  | 2.90   | 2.70  | 2.50  |
| 35 | Phenyl $\alpha$ -naphthylamine, weight percent                     | 0.20  | 0.20  | 0.20   | 0.20  | 0.20  |
|    | Mineral lubricating oil of 80 SSU at 210° F., weight percent       | 91.41 | 91.56 | 91.98  | 92.34 | 92.70 |
| 40 | Max. Temp. of Preparation, ° F.                                    | 320   | 320   | 320    | 320   | 320   |
|    | Mol. Ratio of acetic acid to capric acid                           | 6/1   | 10/1  | 12.5/1 | 15/1  | 19/1  |
| 45 | Properties:                                                        |       |       |        |       |       |
|    | Appearance                                                         | (2)   | (3)   | (3)    | (3)   | (3)   |
|    | Viscosity SSU at 100° F.                                           | 1,800 | 1,603 | 1,485  | 1,492 | 1,431 |
|    | Al nent test, weights carried                                      | 4     | 4     | 6      | 6     | 7     |
|    | 4-ball wear test, scar diam. mm. (1,800 r.p.m.-10 kg.-77° F.-1 hr) | 0.32  | 0.29  | 0.23   | 0.24  | 0.23  |
|    | Free alkalinity                                                    | 0.05  | 0.05  | 0.05   | 0.05  | 0.05  |
| 50 | Centrifuge test:                                                   |       |       |        |       |       |
|    | 4 hr.-1,500 r.p.m., weight percent solids                          | 1.5   | 1.0   | 0.7    | 0.7   | 0.7   |
|    | 1 percent water                                                    | 20.0  | 10.0  | 2.0    | 2.0   | 5.0   |
|    | Sight glass life in days                                           | 2     | 10    | 40     | 35    | 35    |

<sup>1</sup> Commercial capric acid derived from coconut oil and having a saponification number of about 320.

<sup>2</sup> Thixotropic.

<sup>3</sup> Excellent smooth fluid product.

The free alkalinity of Table II is in terms of NaOH.

The sight glass life test of Table II was carried out by passing the lubricant through the sight glass of a Manzell lubricator containing a 50/50 mixture of water and glycerine at the rate of 1 quart per day.

The centrifuge test was carried out by simply centrifuging the lubricant sample and measuring the sediment. A second centrifuge was carried out by mixing 1 wt. percent water with the lubricant and then centrifuging.

Formulations A and B gave relatively more wear and were less stable as measured by the centrifuge test, particularly in the presence of water. This latter aspect is important because of the likelihood of contamination by condensation during storage. In addition, the sight glass life was poor. This also is important since nearly all marine diesel engines are lubricated by a forced feed system having sight glasses to regulate the lubricant flow.

In many of these systems, the lubricant flows upward through a sight glass containing water and glycerine. In this manner, the lubricant flow can be visually observed as the drops of lubricant pass upward through the water-glycerine mixture and the flow adjusted by a regulating valve. Since there is a sight glass for each cylinder, and

considerable work is involved in cleaning a sight glass, the sight glass life of the lubricant is quite important. Thus, Formulation A would require dismantling and cleaning the sight glasses every two days, while Formulations C, D, and E would operate 35 to 40 days without cleaning the sight glasses.

Formulations C, D, and E, which represent the invention, had better extreme pressure properties, gave less wear, had better storage stability and good sight glass life as compared to Formulations A and B. These comparisons thus demonstrate the criticality of the molar ratio of the two types of acids in forming suitable lubricants.

What is claimed is:

1. A lubricant suitable for lubrication of upper cylinders of marine diesel engines comprising a major amount of mineral lubricating oil, and about 5 to 12 wt. percent dry calcium salts of acetic acid and  $C_7$  to  $C_{10}$  straight chain fatty acid in a molar ratio of said acetic acid to said fatty acid of 11.5:1 to 25:1.

2. A method of lubricating the upper cylinders of marine diesel engines which comprises applying to the pistons of said engines the lubricant of claim 1.

3. A method of preparing the lubricant of claim 1 which comprises neutralizing said acids with lime in oil, followed by dehydration at a temperature of 250° to 350° F.

4. A lubricant according to claim 1, wherein the amount of thickener is within the range of 6 to 8 wt. percent and said molar ratio is about 12.5 to 1 to 19 to 1.

5. A lubricant according to claim 1, wherein said  $C_7$  to  $C_{10}$  acid is derived from coconut oil and has a saponification number of about 320.

10

References Cited in the file of this patent

UNITED STATES PATENTS

15 2,274,675 Earle ----- Mar. 3, 1942  
2,417,428 McLennan ----- Mar. 18, 1947  
2,606,753 Holdstock ----- Aug. 5, 1952

20 OTHER REFERENCES  
NLGI Spokesman, vol. 14, No. 12 (March 1951), pp. 7-23.  
Can. J. Research, vol. 22, sec. B, pp. 76-89, article by Gallay et al.